



US007530907B2

(12) **United States Patent**  
**Sullivan et al.**

(10) **Patent No.:** **US 7,530,907 B2**  
(45) **Date of Patent:** **May 12, 2009**

(54) **GOLF BALLS HAVING A LOW MODULUS HNP LAYER AND A HIGH MODULUS HNP LAYER**

(75) Inventors: **Michael J. Sullivan**, Barrington, RI (US); **Derek A. Ladd**, Acushnet, MA (US); **Edmund A. Hebert**, Mattapoisett, MA (US); **Douglas E. Jones**, Dartmouth, MA (US); **Antonio U. DeSimas**, East Providence, RI (US)

(73) Assignee: **Acushnet Company**, Fairhaven, MA (US)

(\*) Notice: Subject to any disclaimer, the term of this patent is extended or adjusted under 35 U.S.C. 154(b) by 0 days.

(21) Appl. No.: **12/125,226**

(22) Filed: **May 22, 2008**

(65) **Prior Publication Data**

US 2008/0220902 A1 Sep. 11, 2008

**Related U.S. Application Data**

(63) Continuation-in-part of application No. 12/102,515, filed on Apr. 14, 2008, which is a continuation of application No. 11/694,029, filed on Mar. 30, 2007, now Pat. No. 7,357,736, which is a continuation-in-part of application No. 11/353,563, filed on Feb. 14, 2006, now Pat. No. 7,458,904.

(51) **Int. Cl.**  
**A63B 37/08** (2006.01)

(52) **U.S. Cl.** ..... 473/354

(58) **Field of Classification Search** ..... 473/354, 473/373, 374, 376

See application file for complete search history.

(56) **References Cited**

**U.S. PATENT DOCUMENTS**

5,779,562 A \* 7/1998 Melvin et al. ..... 473/373  
5,885,172 A \* 3/1999 Hebert et al. ..... 473/354  
7,458,904 B2 \* 12/2008 Sullivan et al. ..... 473/354

\* cited by examiner

*Primary Examiner*—Raeann Trimew

(74) *Attorney, Agent, or Firm*—Mandi B. Milbank

(57) **ABSTRACT**

The present invention is directed to golf balls comprising a fluid-filled center surrounded by an outer core, wherein the outer core comprises a layer formed from a low modulus HNP composition and a layer formed from a high modulus HNP composition. The present invention is not limited by which outer core layer is formed from the low modulus HNP composition and which layer is formed from the high modulus HNP composition, so long as both layers are present in the outer core of the golf ball. Low modulus HNP compositions of the present invention comprise a highly neutralized acid copolymer having a modulus of from 1,000 psi to 50,000 psi. High modulus HNP compositions of the present invention comprise a highly neutralized acid copolymer having a modulus of from 25,000 psi to 150,000 psi.

**18 Claims, No Drawings**

## 1

**GOLF BALLS HAVING A LOW MODULUS  
HNP LAYER AND A HIGH MODULUS HNP  
LAYER**

CROSS-REFERENCE TO RELATED  
APPLICATIONS

This application is a continuation-in-part of U.S. patent application Ser. No. 12/102,515, filed Apr. 14, 2008, which is a continuation of U.S. patent application Ser. No. 11/694,029, filed Mar. 30, 2007, now U.S. Pat. No. 7,357,736, the entire disclosures of which are hereby incorporated herein by reference. This application is also a continuation-in-part of U.S. patent application Ser. No. 11/353,563, filed Feb. 14, 2006 now U.S. Pat. No. 7,458,904, the entire disclosure of which is hereby incorporated herein by reference.

FIELD OF THE INVENTION

The present invention is directed to golf balls comprising a fluid-filled center surrounded by an outer core, wherein the outer core comprises a layer formed from a low modulus HNP composition and a layer formed from a high modulus HNP composition. The present invention is not limited by which outer core layer is formed from the low modulus HNP composition and which outer core layer is formed from the high modulus HNP composition, so long as both layers are present in the outer core of the golf ball.

BACKGROUND OF THE INVENTION

Conventional golf balls can be divided into two general classes: solid and wound. Solid golf balls include one-piece, two-piece (i.e., single layer core and single layer cover), and multi-layer (i.e., solid core of one or more layers and/or a cover of one or more layers) golf balls. Wound golf balls typically include a solid, hollow, or fluid-filled center, surrounded by a tensioned elastomeric material, and a cover.

Golf ball core and cover layers are typically constructed with polymer compositions including, for example, polybutadiene rubber, polyurethanes, polyamides, ionomers, and blends thereof. Ionomers, particularly ethylene-based ionomers, are a preferred group of polymers for golf ball layers because of their toughness, durability, and wide range of hardness values.

Golf ball compositions comprising highly neutralized acid polymers are known. For example, U.S. Patent Application Publication No. 2003/0130434, the entire disclosure of which is hereby incorporated herein by reference, discloses melt-processible, highly-neutralized ethylene acid copolymers and process for making them by incorporating an aliphatic, mono-functional organic acid in the acid copolymer and then neutralizing greater than 90% of all the acid groups present. The use of such compositions in various golf ball layers is disclosed. Also, U.S. Patent Application Publication No. 2005/0148725, the entire disclosure of which is hereby incorporated herein by reference, discloses a highly-resilient thermoplastic composition comprising (a) an acid copolymer, (b) a salt of a high molecular weight, monomeric organic acid; (c) a thermoplastic resin; (d) a cation source; and (e) optionally, a filler. The reference also discloses one-piece, two-piece, three-piece, and multi-layered golf balls comprising the highly-resilient thermoplastic composition.

While various uses for highly neutralized acid polymers in golf balls have been discovered, there is a need in the industry to broaden the applicability of highly neutralized acid polymers to particular golf ball constructions having desirable

## 2

spin, feel, and COR properties. The present invention provides such golf ball constructions through the use of a layer formed from a low modulus HNP composition and a layer formed from a high modulus HNP composition.

5

SUMMARY OF THE INVENTION

In one embodiment, the present invention is directed to a golf ball comprising a core and a cover, wherein the core comprises a fluid mass at the center, a first outer core layer surrounding the fluid mass, and a second outer core layer surrounding the first outer core layer. The first outer core layer is solid, non-wound, and formed from a low modulus HNP composition, and the second outer core layer is solid, non-wound and formed from a high modulus HNP composition. The low modulus HNP composition comprises a highly neutralized ethylene/(meth)acrylic acid/alkyl (meth)acrylate copolymer having a modulus of from 1,000 psi to 50,000 psi. The high modulus HNP composition comprises a highly neutralized ethylene/(meth)acrylic acid copolymer having a modulus of from 25,000 psi to 150,000 psi. The modulus of the highly neutralized copolymer of the low modulus HNP composition is at least 10% less than the modulus of the highly neutralized copolymer of the high modulus HNP composition.

In another embodiment, the present invention is directed to a golf ball comprising a core and a cover, wherein the core comprises a fluid mass at the center, a first outer core layer surrounding the fluid mass, and a second outer core layer surrounding the first outer core layer. The first outer core layer is solid, non-wound, and formed from a high modulus HNP composition, and the second outer core layer is solid, non-wound and formed from a low modulus HNP composition. The high modulus HNP composition comprises a highly neutralized ethylene/(meth)acrylic acid copolymer having a modulus of from 25,000 psi to 150,000 psi. The low modulus HNP composition comprises a high neutralized ethylene/(meth)acrylic acid/alkyl (meth)acrylate copolymer having a modulus of from 1,000 psi to 50,000 psi. The modulus of the highly neutralized copolymer of the low modulus HNP composition is at least 10% less than the modulus of the highly neutralized copolymer of the high modulus HNP composition.

45 DETAILED DESCRIPTION OF THE INVENTION

Golf balls of the present invention have at least two layers formed from highly neutralized acid polymer ("HNP") compositions. More particularly, golf balls of the present invention have at least one layer formed from a low modulus HNP composition, and at least one layer formed from a high modulus HNP composition.

As used herein, "highly neutralized acid polymer" refers to an acid polymer after at least 80%, preferably at least 90%, 55 more preferably at least 95%, and even more preferably 100%, of the acid groups of the acid polymer are neutralized.

For purposes of the present disclosure, material hardness is measured according to ASTM D2240 and generally involves measuring the hardness of a flat "slab" or "button" formed of the material. It should be understood that there is a fundamental difference between "material hardness" and "hardness as measured directly on a golf ball." Hardness as measured directly on a golf ball (or other spherical surface) typically results in a different hardness value than material hardness. This difference in hardness values is due to several factors including, but not limited to, ball construction (i.e., core type, number of core and/or cover layers, etc.), ball (or

sphere) diameter, and the material composition of adjacent layers. It should also be understood that the two measurement techniques are not linearly related and, therefore, one hardness value cannot easily be correlated to the other. Unless stated otherwise, the hardness values given herein for cover materials are material hardness values measured according to ASTM D2240, with all values reported following 10 days of aging at 50% relative humidity and 23° C.

The surface hardness of a golf ball layer is obtained from the average of a number of measurements taken from opposing hemispheres of a core, taking care to avoid making measurements on the parting line of the core or on surface defects, such as holes or protrusions. Hardness measurements are made pursuant to ASTM D-2240 "Indentation Hardness of Rubber and Plastic by Means of a Durometer." Because of the curved surface, care must be taken to insure that the golf ball or golf ball subassembly is centered under the durometer indentor before a surface hardness reading is obtained. A calibrated, digital durometer, capable of reading to 0.1 hardness units is used for all hardness measurements and is set to take hardness readings at 1 second after the maximum reading is obtained. The digital durometer must be attached to, and its foot made parallel to, the base of an automatic stand, such that the weight on the durometer and attack rate conform to ASTM D-2240.

As used herein, "modulus" refers to flexural modulus as measured using a standard flex bar according to ASTM D790-B.

#### Low Modulus HNP Composition

Low modulus HNP compositions of the present invention comprise at least one low modulus HNP having a modulus within the range having a lower limit of 1,000 or 5,000 or 10,000 psi and an upper limit of 17,000 or 25,000 or 28,000 or 30,000 or 35,000 or 45,000 or 50,000 or 55,000 psi. In a preferred embodiment, the modulus of the low modulus HNP is at least 10% less, or at least 20% less, or at least 25% less, or at least 30% less, or at least 35% less, than the modulus of the high modulus HNP.

Low modulus HNPs of the present invention are salts of acid copolymers. It is understood that the low modulus HNP may be a blend of two or more low modulus HNPs. The acid copolymer of the low modulus HNP is an O/X/Y-type copolymer, wherein O is an  $\alpha$ -olefin, X is a  $C_3$ - $C_8$   $\alpha,\beta$ -ethylenically unsaturated carboxylic acid, and Y is a softening monomer. O is preferably ethylene. X is preferably selected from (meth)acrylic acid, ethacrylic acid, maleic acid, crotonic acid, fumaric acid, and itaconic acid. (Meth)acrylic acid is particularly preferred. As used herein, "(meth) acrylic acid" means methacrylic acid and/or acrylic acid. Likewise, "(meth)acrylate" means methacrylate and/or acrylate. Y is preferably an alkyl (meth)acrylate, wherein the alkyl groups have from 1 to 8 carbon atoms. Preferred O/X/Y-type copolymers are those wherein O is ethylene, X is (meth) acrylic acid, and Y is selected from (meth) acrylate, n-butyl (meth) acrylate, isobutyl (meth) acrylate, methyl (meth) acrylate, and ethyl (meth) acrylate. Particularly preferred O/X/Y-type copolymers are ethylene/(meth) acrylic acid/n-butyl acrylate, ethylene/(meth) acrylic acid/methyl acrylate, and ethylene/(meth) acrylic acid/ethyl acrylate.

The acid copolymer of the low modulus HNP typically includes the  $\alpha$ -olefin in an amount of at least 15 wt %, or at least 25 wt %, or at least 40 wt %, or at least 60 wt %, based on the total weight of the acid copolymer. The amount of  $C_3$ - $C_8$   $\alpha,\beta$ -ethylenically unsaturated carboxylic acid in the acid copolymer is typically within the range having a lower limit of 1 or 4 or 6 or 8 or 10 or 15 wt % and an upper limit of

20 or 35 or 40 wt %, based on the total weight of the acid copolymer. The amount of softening monomer in the acid copolymer is typically within the range having a lower limit of 1 or 3 or 5 or 11 or 15 or 20 wt % and an upper limit of 23 or 25 or 30 or 35 or 50 wt %, based on the total weight of the acid copolymer.

Particularly suitable acid copolymers of the low modulus HNP include very low modulus ionomer- ("VLM-") type ethylene-acid polymers, such as Surlyn® 6320, Surlyn® 8120, Surlyn® 8320, and Surlyn® 9320. Surlyn® ionomers are commercially available from E. I. du Pont de Nemours and Company. Also suitable are DuPont® HPF 1000 and DuPont® HPF 2000, ionomeric materials commercially available from E. I. du Pont de Nemours and Company.

Additional suitable acid copolymers of the low modulus HNP are disclosed, for example, in U.S. Patent Application Publication Nos. 2005/0148725, 2005/0020741, 2004/0220343, and 2003/0130434, and U.S. Pat. Nos. 5,691,418, 6,562,906, 6,653,382, 6,777,472, 6,762,246, and 6,815,480, the entire disclosures of which are hereby incorporated herein by reference.

In a preferred embodiment, the low modulus HNP is formed by reacting an acid copolymer, which is optionally partially neutralized, with a sufficient amount of cation source, in the presence of a high molecular weight organic acid or salt thereof, such that at least 80%, preferably at least 90%, more preferably at least 95%, and even more preferably 100%, of all acid groups present are neutralized. The acid copolymer can be reacted with the high molecular weight organic acid or salt thereof and the cation source simultaneously, or the acid copolymer can be reacted with the high molecular weight organic acid prior to the addition of the cation source.

Suitable high molecular weight organic acids are aliphatic organic acids, aromatic organic acids, saturated monofunctional organic acids, unsaturated monofunctional organic acids, multi-unsaturated monofunctional organic acids, and dimerized derivatives thereof. Particular examples of suitable organic acids include, but are not limited to, caproic acid, caprylic acid, capric acid, lauric acid, stearic acid, behenic acid, erucic acid, oleic acid, linoleic acid, myristic acid, benzoic acid, palmitic acid, phenylacetic acid, naphthalenoic acid, dimerized derivatives thereof, and combinations thereof. Salts of high molecular weight organic acids comprise the salts, particularly the barium, lithium, sodium, zinc, bismuth, chromium, cobalt, copper, potassium, stontium, titanium, tungsten, magnesium, and calcium salts, of aliphatic organic acids, aromatic organic acids, saturated monofunctional organic acids, unsaturated monofunctional organic acids, multi-unsaturated monofunctional organic acids, dimerized derivatives thereof, and combinations thereof. Suitable organic acids and salts thereof are more fully described, for example, in U.S. Pat. No. 6,756,436, the entire disclosure of which is hereby incorporated herein by reference.

Suitable cation sources include metal ions and compounds of alkali metals, alkaline earth metals, and transition metals; metal ions and compounds of rare earth elements; silicone, silane, and silicate derivatives and complex ligands; and combinations thereof. Preferred cation sources are metal ions and compounds of magnesium, sodium, potassium, cesium, calcium, barium, manganese, copper, zinc, tin, lithium, and rare earth metals. The acid copolymer may be at least partially neutralized prior to contacting the acid copolymer with the cation source to form the low modulus HNP. Methods of preparing ionomers are well known, and are disclosed, for example, in U.S. Pat. No. 3,264,272, the entire disclosure of

which is hereby incorporated herein by reference. The acid copolymer can be a direct copolymer wherein the polymer is polymerized by adding all monomers simultaneously, as disclosed, for example, in U.S. Pat. No. 4,351,931, the entire disclosure of which is hereby incorporated herein by reference. Alternatively, the acid copolymer can be a graft copolymer wherein a monomer is grafted onto an existing polymer, as disclosed, for example, in U.S. Patent Application Publication No. 2002/0013413, the entire disclosure of which is hereby incorporated herein by reference.

Low modulus HNP compositions of the present invention optionally contain one or more melt flow modifiers. The amount of melt flow modifier in the composition is readily determined such that the melt flow index of the composition is at least 0.1 g/10 min, preferably from 0.5 g/10 min to 10.0 g/10 min, and more preferably from 1.0 g/10 min to 6.0 g/10 min, as measured using ASTM D-1238, condition E, at 190° C., using a 2160 gram weight.

Suitable melt flow modifiers include, but are not limited to, high molecular weight organic acids and salts thereof, polyamides, polyesters, polyacrylates, polyurethanes, polyethers, polyureas, polyhydric alcohols, and combinations thereof. Suitable organic acids are aliphatic organic acids, aromatic organic acids, saturated mono-functional organic acids, unsaturated monofunctional organic acids, multi-unsaturated mono-functional organic acids, and dimerized derivatives thereof. Particular examples of suitable organic acids include, but are not limited to, caproic acid, caprylic acid, capric acid, lauric acid, stearic acid, behenic acid, erucic acid, oleic acid, linoleic acid, myristic acid, benzoic acid, palmitic acid, phenylacetic acid, naphthalenoic acid, dimerized derivatives thereof. Suitable organic acids are more fully described, for example, in U.S. Pat. No. 6,756,436, the entire disclosure of which is hereby incorporated herein by reference.

Additional melt flow modifiers suitable for use in compositions of the present invention, include the non-fatty acid melt flow modifiers described in copending U.S. patent application Ser. Nos. 11/216,725 and 11/216,726, the entire disclosures of which are hereby incorporated herein by reference.

Low modulus HNP compositions of the present invention optionally include additive(s) and/or filler(s) in an amount of 50 wt % or less, or 30 wt % or less, or 15 wt % or less, based on the total weight of the low modulus HNP composition. Suitable additives and fillers include, but are not limited to, chemical blowing and foaming agents, optical brighteners, coloring agents, fluorescent agents, whitening agents, UV absorbers, light stabilizers, defoaming agents, processing aids, mica, talc, nano-fillers, antioxidants, stabilizers, softening agents, fragrance components, plasticizers, impact modifiers,  $TiO_2$ , acid copolymer wax, surfactants, and fillers, such as zinc oxide, tin oxide, barium sulfate, zinc sulfate, calcium oxide, calcium carbonate, zinc carbonate, barium carbonate, clay, tungsten, tungsten carbide, silica, lead silicate, regrind (recycled material), and mixtures thereof. Suitable additives are more fully described in, for example, U.S. Patent Application Publication No. 2003/0225197, the entire disclosure of which is hereby incorporated herein by reference.

Low modulus HNP compositions of the present invention optionally contain a high modulus HNP.

Low modulus HNP compositions of the present invention preferably have a hardness within the range having a lower limit of 40 or 50 or 55 Shore C and an upper limit of 70 or 80 or 87 Shore C.

In a particular embodiment, the low modulus HNP composition has a moisture vapor transmission rate of 8 g-mil/100 in<sup>2</sup>/day or less (i.e., 3.2 g-mm/m<sup>2</sup>·day or less), or 5 g-mil/100

in<sup>2</sup>/day or less (i.e., 2.0 g-mm/m<sup>2</sup>·day or less), or 3 g-mil/100 in<sup>2</sup>/day or less (i.e., 1.2 g-mm/m<sup>2</sup>·day or less), or 2 g-mil/100 in<sup>2</sup>/day or less (i.e., 0.8 g-mm/m<sup>2</sup>·day or less), or 1 g-mil/100 in<sup>2</sup>/day or less (i.e., 0.4 g-mm/m<sup>2</sup>·day or less), or less than 1 g-mil/100 in<sup>2</sup>/day (i.e., less than 0.4 g-mm/m<sup>2</sup>·day). As used herein, moisture vapor transmission rate ("MVTR") is given in g-mil/100 in<sup>2</sup>/day, and is measured at 20° C. and according to ASTM F 1249-99. In a preferred aspect of this embodiment, the low modulus HNP composition comprises a low modulus HNP prepared using a cation source which is less hydrophilic than conventional magnesium-based cation sources. Suitable moisture resistant HNP compositions are disclosed, for example, in U.S. Patent Application Publication Nos. 2005/0267240, 2006/0106175 and 2006/0293464, the entire disclosures of which are hereby incorporated herein by reference.

In another particular embodiment, a sphere formed from the low modulus HNP composition has a compression of 80 or less, or 70 or less, or 65 or less, or 60 or less, or 50 or less, or 40 or less, or 30 or less, or 20 or less.

Low modulus HNP compositions of the present invention are not limited by any particular method or any particular equipment for making the compositions. In a preferred embodiment, the composition is prepared by the following process. The acid polymer(s), preferably a VLMI-type ethylene-acid terpolymer, high molecular weight organic acid(s) or salt(s) thereof, and optionally additive(s)/filler(s) are simultaneously or individually fed into a melt extruder, such as a single or twin screw extruder. A suitable amount of cation source is simultaneously or subsequently added such that at least 80%, preferably at least 90%, more preferably at least 95%, and even more preferably 100%, of all acid groups present are neutralized. The acid polymer may be at least partially neutralized prior to the above process. The components are intensively mixed prior to being extruded as a strand from the die-head.

Low modulus HNP compositions of the present invention may be blended with one or more additional polymers, such as thermoplastic polymers and elastomers. Examples of thermoplastic polymers suitable for blending include, but are not limited to, bimodal ionomers (e.g., as disclosed in U.S. Patent Application Publication No. 2004/0220343 and U.S. Pat. Nos. 6,562,906, 6,762,246 and 7,273,903, the entire disclosures of which are hereby incorporated herein by reference), ionomers modified with rosins (e.g., as disclosed in U.S. Patent Application Publication No. 2005/0020741, the entire disclosure of which is hereby incorporated by reference), soft and resilient ethylene copolymers (e.g., as disclosed U.S. Patent Application Publication No. 2003/0114565, the entire disclosure of which is hereby incorporated herein by reference) polyolefins, polyamides, polyesters, polyethers, polycarbonates, polysulfones, polyacetals, polylactones, acrylonitrile-butadiene-styrene resins, polyphenylene oxide, polyphenylene sulfide, styrene-acrylonitrile resins, styrene maleic anhydride, polyimides, aromatic polyketones, ionomers and ionomeric precursors, acid copolymers, conventional HNPs, polyurethanes, grafted and non-grafted metallocene-catalyzed polymers, single-site catalyst polymerized polymers, high crystalline acid polymers, cationic ionomers, and combinations thereof. Particular polyolefins suitable for blending include one or more, linear, branched, or cyclic,  $C_2$ - $C_{40}$  olefins, particularly polymers comprising ethylene or propylene copolymerized with one or more  $C_2$ - $C_{40}$  olefins,  $C_3$ - $C_{20}$   $\alpha$ -olefins, or  $C_3$ - $C_{10}$   $\alpha$ -olefins. Particular conventional HNPs suitable for blending include, but are not limited to, one or more of the HNPs disclosed in U.S. Pat. Nos. 6,756,436, 6,894,098, and 6,953,820, the entire disclosures

of which are hereby incorporated herein by reference. Examples of elastomers suitable for blending with the invention polymers include natural and synthetic rubbers, including, but not limited to, ethylene propylene rubber ("EPR"), ethylene propylene diene rubber ("EPDM"), styrenic block copolymer rubbers (such as SI, SIS, SB, SBS, SIBS, and the like, where "S" is styrene, "I" is isobutylene, and "B" is butadiene), butyl rubber, halobutyl rubber, copolymers of isobutylene and para-alkylstyrene, halogenated copolymers of isobutylene and para-alkylstyrene, natural rubber, polyisoprene, copolymers of butadiene with acrylonitrile, polychloroprene, alkyl acrylate rubber, chlorinated isoprene rubber, acrylonitrile chlorinated isoprene rubber, and polybutadiene rubber (cis and trans). Additional suitable blend polymers include those described in U.S. Pat. No. 5,981,658, for example at column 14, lines 30 to 56, the entire disclosure of which is hereby incorporated herein by reference. The blends described herein may be produced by post-reactor blending, by connecting reactors in series to make reactor blends, or by using more than one catalyst in the same reactor to produce multiple species of polymer. The polymers may be mixed prior to being put into an extruder, or they may be mixed in an extruder.

Particularly suitable low modulus HNP compositions include, but are not limited to, the highly-resilient thermoplastic compositions disclosed in U.S. Patent Application Publication No. 2005/0148725; the highly-neutralized ethylene copolymers disclosed in U.S. Pat. Nos. 6,653,382 and 6,777,472, and U.S. Patent Application Publication No. 2003/0130434; and the highly-resilient thermoplastic elastomer compositions disclosed in U.S. Pat. No. 6,815,480; the entire disclosures of which are hereby incorporated herein by reference.

#### High Modulus HNP Composition

High modulus HNP compositions of the present invention comprise at least one high modulus HNP having a modulus within the range having a lower limit of 25,000 or 27,000 or 30,000 or 40,000 or 45,000 or 50,000 or 55,000 or 60,000 psi and an upper limit of 72,000 or 75,000 or 100,000 or 150,000 psi.

High modulus HNPs of the present invention are salts of acid copolymers. It is understood that the high modulus HNP may be a blend of two or more high modulus HNPs. Preferred acid copolymers are copolymers of an  $\alpha$ -olefin and a C<sub>3</sub>-C<sub>8</sub>  $\alpha$ , $\beta$ -ethylenically unsaturated carboxylic acid. The acid is typically present in the acid copolymer in an amount within the range having a lower limit of 1 or 10 or 12 or 15 or 20 wt % and an upper limit of 25 or 30 or 35 or 40 wt %, based on the total weight of the acid copolymer. The  $\alpha$ -olefin is preferably selected from ethylene and propylene. The acid is preferably selected from (meth) acrylic acid, ethacrylic acid, maleic acid, crotonic acid, fumaric acid, and itaconic acid. (Meth) acrylic acid is particularly preferred. In a preferred embodiment, the high modulus HNP has a higher level of acid than the low modulus HNP.

Suitable acid copolymers include partially neutralized acid polymers. Examples of suitable partially neutralized acid polymers include, but are not limited to, Surlyn® ionomers, commercially available from E. I. du Pont de Nemours and Company; AClyn® ionomers, commercially available from Honeywell International Inc.; and Iotek® ionomers, commercially available from ExxonMobil Chemical Company. Also suitable are DuPont® HPF 1000 and DuPont® HPF 2000, ionomer materials commercially available from E. I. du Pont de Nemours and Company. Additional suitable acid polymers are more fully described, for example, in U.S. Pat.

Nos. 6,562,906, 6,762,246, and 6,953,820 and U.S. Patent Application Publication Nos. 2005/0049367, 2005/0020741, and 2004/0220343, the entire disclosures of which are hereby incorporated herein by reference.

- 5 In a preferred embodiment, the high modulus HNP is formed by reacting an acid copolymer with a sufficient amount of cation source such that at least 80%, preferably at least 90%, more preferably at least 95%, and even more preferably 100%, of all acid groups present are neutralized. 10 Suitable cation sources include metal ions and compounds of alkali metals, alkaline earth metals, and transition metals; metal ions and compounds of rare earth elements; silicone, silane, and silicate derivatives and complex ligands; and combinations thereof. Preferred cation sources are metal ions and compounds of magnesium, sodium, potassium, cesium, calcium, barium, manganese, copper, zinc, tin, lithium, and rare earth metals. Metal ions and compounds of calcium and magnesium are particularly preferred. The acid copolymer may be at least partially neutralized prior to contacting the acid 15 copolymer with the cation source to form the high modulus HNP. As previously stated, methods of preparing ionomers, and the acid copolymers on which ionomers are based, are disclosed, for example, in U.S. Pat. Nos. 3,264,272, and 4,351,931, and U.S. Patent Application Publication No. 2002/20 0013413.

High modulus HNP compositions of the present invention optionally contain one or more melt flow modifiers. The amount of melt flow modifier in the composition is readily determined such that the melt flow index of the composition 30 is at least 0.1 g/10 min, preferably from 0.5 g/10 min to 10.0 g/10 min, and more preferably from 1.0 g/10 min to 6.0 g/10 min, as measured using ASTM D-1238, condition E, at 190° C., using a 2160 gram weight.

Suitable melt flow modifiers include, but are not limited to, 35 high molecular weight organic acids and salts thereof, polyamides, polyesters, polyacrylates, polyurethanes, polyethers, polyureas, polyhydric alcohols, and combinations thereof. Suitable organic acids are aliphatic organic acids, aromatic organic acids, saturated mono-functional organic acids, 40 unsaturated monofunctional organic acids, multi-unsaturated mono-functional organic acids, and dimerized derivatives thereof. Particular examples of suitable organic acids include, but are not limited to, caproic acid, caprylic acid, capric acid, lauric acid, stearic acid, behenic acid, erucic acid, oleic acid, linoleic acid, myristic acid, benzoic acid, palmitic acid, phenylacetic acid, naphthalenoic acid, dimerized derivatives thereof. Suitable organic acids are more fully described, for 45 example, in U.S. Pat. No. 6,756,436, the entire disclosure of which is hereby incorporated herein by reference.

Additional melt flow modifiers suitable for use in compositions of the present invention, include the non-fatty acid melt flow modifiers described in copending U.S. patent application Ser. Nos. 11/216,725 and 11/216,726, the entire disclosures of which are hereby incorporated herein by reference.

High modulus HNP compositions of the present invention 55 optionally include additive(s) and/or filler(s) in an amount within the range having a lower limit of 0 or 5 or 10 wt %, and an upper limit of 25 or 30 or 50 wt %, based on the total weight of the high modulus HNP composition. Suitable additives and fillers include those previously described as suitable for the low modulus HNP compositions of the present invention.

In addition to the high modulus HNP, optional melt flow 60 modifier(s), and optional additive(s) and/or filler(s), the high modulus HNP composition of the present invention may contain a low modulus HNP.

In a particular embodiment, the high modulus HNP composition has an MVTR of 8 g-mil/100 in<sup>2</sup>/day or less (i.e., 3.2 g-mm/m<sup>2</sup>·day or less), or 5 g-mil/100 in<sup>2</sup>/day or less (i.e., 2.0 g-mm/m<sup>2</sup>·day or less), or 3 g-mil/100 in<sup>2</sup>/day or less (i.e., 1.2 g-mm/m<sup>2</sup>·day or less), or 2 g-mil/100 in<sup>2</sup>/day or less (i.e., 0.8 g-mm/m<sup>2</sup>·day or less), or 1 g-mil/100 in<sup>2</sup>/day or less (i.e., 0.4 g-mm/m<sup>2</sup>·day or less), or less than 1 g-mil/100 in<sup>2</sup>/day (i.e., less than 0.4 g-mm/m<sup>2</sup>·day). In a preferred aspect of this embodiment, the high modulus HNP composition comprises a high modulus HNP prepared using a cation source which is less hydrophilic than conventional magnesium-based cation sources. Suitable moisture resistant HNP compositions are disclosed, for example, in copending U.S. patent application Ser. No. 11/270,066 and U.S. Patent Application Publication No. 2005/0267240, the entire disclosures of which are hereby incorporated herein by reference.

In another particular embodiment, a sphere formed from the high modulus HNP composition has a compression of 70 or greater, or 80 or greater, or a compression within a range having a lower limit of 70 or 80 or 90 or 100 and an upper limit of 110 or 130 or 140.

High modulus HNP compositions of the present invention are not limited by any particular method or any particular equipment for making the compositions. In a preferred embodiment, the composition is prepared by the following process. The acid polymer(s), preferably an ethylene/(meth) acrylic acid copolymer, optional melt flow modifier(s), and optional additive(s)/filler(s) are simultaneously or individually fed into a melt extruder, such as a single or twin screw extruder. A suitable amount of cation source is then added such that at least 80%, preferably at least 90%, more preferably at least 95%, and even more preferably 100%, of all acid groups present are neutralized. The acid polymer may be at least partially neutralized prior to the above process. The components are intensively mixed prior to being extruded as a strand from the die-head.

In another preferred embodiment, the high modulus HNP composition is formed by combining a low modulus HNP with a sufficient amount of one or more additional material(s), including, but not limited to, additives, fillers, and polymeric materials, to increase the modulus such that the resulting composition has a modulus as described above for the high modulus HNP.

HNP compositions of the present invention may be blended with one or more additional polymers, such as thermoplastic polymers and elastomers. Examples of thermoplastic polymers and elastomers suitable for blending include those previously described as suitable for blending with the low modulus HNP compositions of the present invention.

#### Golf Ball Applications

Golf balls of the present invention include a center, an outer core having at least two layers, and a cover. The center is solid, semi-solid, hollow, powder-filled or fluid-filled. Preferably, the center is fluid-filled.

As used herein, "fluid" refers to a gas, liquid, gel, paste, or the like, or a combination thereof. Suitable fluids include a wide variety of materials, including solutions and gases, as well as liquids having low coefficient of thermal expansion and/or high boiling points. The fluid is preferably selected from gases (and may be pressurized and/or non-reactive), such as air, nitrogen, helium, argon, neon, carbon dioxide, nitrous oxide, and mixtures thereof; water; polyols, such as glycerine, ethylene glycol, and the like; paste; foams; oil; water solutions, such as salt in water, corn syrup, salt in water and corn syrup, or glycol and water; and combinations thereof. The fluid can also include pastes, colloidal suspen-

sions, such as clay, barytes, carbon black in water or other liquid, or salt in water/glycol mixtures; gels, such as gelatin gels, hydrogels, water/methyl cellulose gels and gels comprised of copolymer rubber based materials such as styrene-butadiene-styrene rubber and paraffinic and/or naphthenic oil; or melts including waxes and hot melts. Hot-melts are materials which at or about normal room temperature are solid but at elevated temperatures become liquid. The fluid can also be a reactive liquid system which, when combined, forms a solid. Examples of suitable reactive liquids, include, but are not limited to, silicate gels, agar gels, peroxide cured polyester resins, two part epoxy resin systems, and peroxide cured liquid polybutadiene rubber compositions. Suitable liquids for use in the center are further disclosed, for example, in U.S. Pat. Nos. 6,200,230, 5,683,312, and 5,150,906, the entire disclosures of which are hereby incorporated herein by reference.

The fluid can be varied to modify the performance parameters of the ball, such as the moment of inertia. For example, the fluid-filled center preferably comprises a material that has a high specific gravity for high spin rate golf balls and a material that has a low specific gravity for low spin rate golf balls. The specific gravity of the fluid for low specific gravity centers is preferably 1.2 or less, or from 0.90 to 1.2, or from 1.15 to 1.2; and for high specific gravity centers is preferably greater than 1.2, or from 1.21 to 1.70, or from 1.3 to 1.55. Additionally, the fluid-filled center preferably comprises a material with a low viscosity for high spin rate golf balls having and a material having a high viscosity for low spin rate golf balls. The viscosity of the fluid for low viscosity centers is preferably less than 100 cps, or 10 cps or less; and for high viscosity centers is preferably 100 cps or greater, or from 100 to 1500 cps.

Known techniques may be used to modify the frictional drag of the fluid inside the center. For example, a texture may be added to the inner surface of the layer immediately surrounding the fluid. The texture can be in the form of dimples, nubs, paddles, fingers, or the like, extending into the center of the core of the golf ball, or can be in the form of grooves cut or molded into the inner surface of the immediately surrounding layer. Individual textures can themselves be modified by increasing or decreasing their size or depth, or alternating their placement or number. Additionally, protrusions of varying sizes or shapes can be used on the inner surface of the immediately surrounding layer. Such modifications and their effect on golf ball properties, such as spin decay, are further disclosed in U.S. Patent Application Publication No. 2006/0142096, the entire disclosure of which is hereby incorporated herein by reference.

The fluid-filled center preferably has a diameter within a range having a lower limit of 0.25 or 0.50 or 0.60 or 0.75 or 0.80 or 1.00 or 1.10 inches and an upper limit of 1.300 or 1.350 or 1.400 or 1.500 or 1.510 or 1.530 or 1.550 or 1.570 or 1.580 inches.

Golf balls having a fluid-filled center are further disclosed, for example, in U.S. Patent Application Publication No. 2006/0142096, the entire disclosure of which is hereby incorporated by reference.

The center is surrounded by a first outer core layer, and the first outer core layer is surrounded by a second core layer. In one embodiment, the first outer core layer is formed from a low modulus HNP composition, and the second outer core layer is formed from a high modulus HNP composition. In another embodiment, the first outer core layer is formed from a high modulus HNP composition, and the second outer core layer is formed from a low modulus HNP composition.

## 11

Golf balls having a layer formed from a low modulus HNP composition and a layer formed from a high modulus HNP composition are further disclosed, for example, in U.S. Pat. No. 7,211,008, the entire disclosure of which is hereby incorporated herein by reference.

The first outer core layer preferably has a thickness within a range having a lower limit of 0.020 or 0.025 or 0.032 or 0.050 or 0.075 or 0.100 or 0.125 inches and an upper limit of 0.150 or 0.175 or 0.200 or 0.220 or 0.250 or 0.280 or 0.300 inches. The second outer core layer preferably has a thickness within a range having a lower limit of 0.020 or 0.025 or 0.032 inches and an upper limit of 0.310 or 0.440 or 0.560 inches. The second outer core layer preferably has a thickness such that the core has an overall diameter within a range having a lower limit of 1.450 or 1.500 or 1.510 or 1.530 or 1.550 inches and an upper limit of 1.560 or 1.570 or 1.580 or 1.590 or 1.600 or 1.620 inches. The first and second outer core layers preferably have a combined thickness within a range having a lower limit of 0.040 inches and an upper limit of 0.560 or 0.800 inches.

Optionally, the golf ball includes a thin shell layer disposed between the center and the first outer core layer. Suitable materials for forming the thin shell layer include, but are not limited to, elastomers, such as thermoset rubber, such as polyisoprene, styrene butadiene, polybutadiene, and combinations thereof, plastics, such as polypropylene and polyethylene; thermoplastic elastomers, such as copolymers of methyl-methacrylate with butadiene and styrene, copolymers of methyl-acrylate with butadiene and styrene, acrylonitrile-styrene copolymers, polyether-ester, polyether-amide, polyurethane; and blends thereof. Particularly suitable are plastic materials having high temperature resistance, such as those disclosed in U.S. Pat. No. 6,616,549, the entire disclosure of which is hereby incorporated herein by reference. Also suitable are acid copolymers, ionomers, and conventional HNPs. Thin shell layers, including materials and constructions, are further disclosed as the "liquid center shell" in U.S. Patent Application Publication No. 2006/0142096, the entire disclosure of which is hereby incorporated herein by reference.

The weight distribution of the core can be varied to achieve certain desired parameters, such as spin rate, compression, and initial velocity.

Golf balls of the present invention include a cover, which may be a single-, dual-, or multi-layer cover. Suitable cover layer materials for the golf balls disclosed herein include, but are not limited to, ionomer resin and blends thereof (particularly Surlyn® ionomer resins), polyurethanes, polyureas, (meth)acrylic acid, thermoplastic rubber polymers, polyethylene, and synthetic or natural vulcanized rubber, such as balata. Suitable commercially available ionomer cover materials include, but are not limited to, Surlyn® ionomer resins and DuPont® HPF 1000 and HPF 2000, commercially available from E. I. du Pont de Nemours and Company; and Iotek® ionomers, commercially available from ExxonMobil Chemical Company.

Particularly suitable outer cover layer materials include relatively soft polyurethanes and polyureas. When used as cover layer materials, polyurethanes and polyureas can be thermoset or thermoplastic. Thermoset materials can be formed into golf ball layers by conventional casting or reaction injection molding techniques. Thermoplastic materials can be formed into golf ball layers by conventional compression or injection molding techniques. Light stable polyureas and polyurethanes are preferred for the outer cover layer material. Additional suitable cover and rubber core materials are disclosed, for example, in U.S. Patent Application Publication No. 2005/0164810, U.S. Pat. No. 5,919,100, and PCT

## 12

Publications WO00/23519 and WO00/29129, the entire disclosures of which are hereby incorporated herein by reference. In embodiments of the present invention wherein a golf ball having a single layer cover is provided, the cover layer material is preferably selected from polyurethane and polyurea. In embodiments of the present invention wherein a golf ball having a dual cover is provided, the inner cover layer is preferably a high modulus thermoplastic, and the outer cover layer is preferably selected from polyurethane and polyurea.

Also suitable are blends of ionomers with thermoplastic elastomers. Suitable ionomer cover materials are further disclosed, for example, in U.S. Pat. Nos. 6,653,382, 6,756,436, 6,894,098, 6,919,393, and 6,953,820, the entire disclosures of which are hereby incorporated by reference. Suitable polyurethane cover materials are further disclosed in U.S. Pat. Nos. 5,334,673, 6,506,851, 6,756,436, and 7,105,623, the entire disclosures of which are hereby incorporated herein by reference. Suitable polyurea cover materials are further disclosed in U.S. Pat. Nos. 5,484,870 and 6,835,794, the entire disclosures of which are hereby incorporated herein by reference. Suitable polyurethane-urea hybrids are blends or copolymers comprising urethane or urea segments as disclosed in U.S. Patent Application Publication No. 2007/0117923, the entire disclosure of which is hereby incorporated herein by reference. Additional suitable cover materials are disclosed, for example, in U.S. Patent Application Publication No. 2005/0164810, U.S. Pat. No. 5,919,100, and PCT Publications WO00/23519 and WO00/29129, the entire disclosures of which are hereby incorporated herein by reference.

In a particular embodiment, the cover is a single layer preferably formed from an ionomer composition. The single layer cover preferably has a surface hardness of 65 Shore D or less, or 60 Shore D or less, or 45 Shore D or less, or 40 Shore D or less, or from 25 Shore D to 40 Shore D, or from 30 Shore D to 40 Shore D and a thickness within a range having a lower limit of 0.010 or 0.015 or 0.020 or 0.025 or 0.030 or 0.055 or 0.060 inches and an upper limit of 0.065 or 0.080 or 0.090 or 0.100 or 0.110 or 0.120 or 0.140 inches. The flexural modulus of the cover, as measured by ASTM D6272-98 Procedure B, is preferably 500 psi or greater, or from 500 psi to 150,000 psi.

In another particular embodiment, the cover is a two-layer cover consisting of an inner cover layer and an outer cover layer. The inner cover layer is preferably formed from an ionomer composition, and preferably has a surface hardness within a range having a lower limit of 30 or 40 or 55 or 60 or 65 Shore D and an upper limit of 66 or 68 or 70 or 75 Shore D, and a thickness within a range having a lower limit of 0.010 or 0.015 or 0.020 or 0.030 inches and an upper limit of 0.035 or 0.040 or 0.045 or 0.050 or 0.055 or 0.075 or 0.080 or 0.110 or 0.120 inches. The outer cover layer is preferably formed from a castable or reaction injection moldable polyurethane, polyurea, or copolymer or hybrid of polyurethane/polyurea.

Such cover material is preferably thermosetting, but may be thermoplastic, and preferably has a surface hardness within a range having a lower limit of 30 or 40 Shore D and an upper limit of 52 or 58 or 62 or 66 or 72 or 75 Shore D. The outer cover layer preferably has a thickness within a range having a lower limit of 0.010 or 0.015 or 0.025 inches and an upper limit of 0.035 or 0.040 or 0.045 or 0.050 or 0.055 or 0.075 or 0.080 or 0.115 inches.

The present invention is not limited by any particular process for forming the golf ball layer(s). It should be understood that the layer(s) can be formed by any suitable technique, including injection molding, compression molding, casting, and reaction injection molding. Reaction injection molding

processes are further disclosed, for example, in U.S. Pat. Nos. 6,083,119, 7,338,391, 7,282,169, 7,281,997 and U.S. Patent Application Publication No. 2006/0247073, the entire disclosures of which are hereby incorporated herein by reference.

In the embodiments disclosed herein, the low modulus HNP composition and/or the high modulus HNP composition, can be either foamed or filled with density adjusting materials to provide desirable golf ball performance characteristics.

HNP compositions of the present invention, in the neat (i.e., unfilled) form, preferably have a specific gravity of from 0.95 g/cc to 0.99 g/cc. Any suitable filler, flake, fiber, particle, or the like, of an organic or inorganic material may be added to the HNP composition to increase or decrease the specific gravity, particularly to adjust the weight distribution within the golf ball, as further disclosed in U.S. Pat. Nos. 6,494,795, 6,547,677, 6,743,123, 7,074,137, and 6,688,991, the entire disclosures of which are hereby incorporated herein by reference.

Golf ball cores of the present invention, typically have an overall core compression of less than 100, or a compression of 87 or less, and preferably have an overall core compression within the range having a lower limit of 20 or 50 or 60 or 65 or 70 and an upper limit of 80 or 85 or 90 or 100 or 110 or 120. Golf balls of the present invention typically have a compression of 120 or less, or a compression within a range having a lower limit of 50 or 60 or 65 or 75 or 80 or 90 and an upper limit of 95 or 100 or 105 or 110 or 115 or 120.

Compression is an important factor in golf ball design. For example, the compression of the core can affect the ball's spin rate off the driver and the feel. As disclosed in Jeff Dalton's *Compression by Any Other Name, Science and Golf IV, Proceedings of the World Scientific Congress of Golf* (Eric Thain ed., Routledge, 2002) ("J. Dalton"), several different methods can be used to measure compression, including Atti compression, Riehle compression, load/deflection measurements at a variety of fixed loads and offsets, and effective modulus. For purposes of the present invention, "compression" refers to Atti compression and is measured according to a known procedure, using an Atti compression test device, wherein a piston is used to compress a ball against a spring. The travel of the piston is fixed and the deflection of the spring is measured. The measurement of the deflection of the spring does not begin with its contact with the ball; rather, there is an offset of approximately the first 1.25 mm (0.05 inches) of the spring's deflection. Very low stiffness cores will not cause the spring to deflect by more than 1.25 mm and therefore have a zero compression measurement. The Atti compression tester is designed to measure objects having a diameter of 42.7 mm (1.68 inches); thus, smaller objects, such as golf ball cores, must be shimmed to a total height of 42.7 mm to obtain an accurate reading. Conversion from Atti compression to Riehle (cores), Riehle (balls), 100 kg deflection, 130-10 kg deflection or effective modulus can be carried out according to the formulas given in J. Dalton.

Golf ball cores of the present invention typically have a coefficient of restitution ("COR") at 125 ft/s of at least 0.75, preferably at least 0.78, and more preferably at least 0.79. Golf balls of the present invention typically have a COR at 125 ft/s of at least 0.75, preferably at least 0.78, and more preferably at least 0.79.

COR, as used herein, is determined according to a known procedure wherein a golf ball or golf ball subassembly (e.g., a golf ball core) is fired from an air cannon at a given velocity (125 ft/s for purposes of the present invention). Ballistic light screens are located between the air cannon and the steel plate to measure ball velocity. As the ball travels toward the steel

plate, it activates each light screen, and the time at each light screen is measured. This provides an incoming transit time period proportional to the ball's incoming velocity. The ball impacts the steel plate and rebounds through the light screens, which again measure the time period required to transit between the light screens. This provides an outgoing transit time period proportional to the ball's outgoing velocity. COR is then calculated as the ratio of the outgoing transit time period to the incoming transit time period,  $COR = T_{out}/T_{in}$ .

Golf balls of the present invention will typically have dimple coverage of 60% or greater, preferably 65% or greater, and more preferably 75% or greater.

The United States Golf Association specifications limit the minimum size of a competition golf ball to 1.680 inches. There is no specification as to the maximum diameter, and golf balls of any size can be used for recreational play. Golf balls of the present invention can have an overall diameter of any size. The preferred diameter of the present golf balls is from 1.680 inches to 1.800 inches. More preferably, the present golf balls have an overall diameter of from 1.680 inches to 1.760 inches, and even more preferably from 1.680 inches to 1.740 inches.

Golf balls of the present invention preferably have a moment of inertia ("MOI") of 70-95 g·cm<sup>2</sup>, preferably 75-93 g·cm<sup>2</sup>, and more preferably 76-90 g·cm<sup>2</sup>. For low MOI embodiments, the golf ball preferably has an MOI of 85 g·cm<sup>2</sup> or less, or 83 g·cm<sup>2</sup> or less. For high MOI embodiment, the golf ball preferably has an MOI of 86 g·cm<sup>2</sup> or greater, or 87 g·cm<sup>2</sup> or greater. MOI is measured on a model MOI-005-104 Moment of Inertia Instrument manufactured by Inertia Dynamics of Collinsville, Conn. The instrument is connected to a PC for communication via a COMM port and is driven by MOI Instrument Software version #1.2.

Thermoplastic layers herein may be treated in such a manner as to create a positive or negative core hardness gradient. The hardness gradient is defined by hardness measurements made at the surface of the layer and radially inward towards the center of the core, typically at 2 mm increments. For purposes of the present invention, "negative" and "positive" refer to the result of subtracting the hardness value at the innermost portion of the golf ball component from the hardness value at the outer surface of the component. For example, if the outer surface of a solid core has a lower hardness value than the center (i.e., the surface is softer than the center), the hardness gradient will be deemed a "negative" gradient. Hardness gradients are disclosed more fully, for example, in U.S. patent application Ser. Nos. 11/832,163, filed on Aug. 1, 2007; 11/939,632, filed on Nov. 14, 2007; 11/939,634, filed on Nov. 14, 2007; 11/939,635, filed on Nov. 14, 2007; and 11/939,637, filed on Nov. 14, 2007; the entire disclosure of each of these references is hereby incorporated herein by reference.

In golf ball layers of the present invention wherein a thermosetting rubber is used, gradient-producing processes and/or gradient-producing rubber formulation may be employed. Gradient-producing processes and formulations are disclosed more fully, for example, in U.S. patent application Ser. Nos. 12/048,665, filed on Mar. 14, 2008; 11/829,461, filed on Jul. 27, 2007; 11/772,903, filed Jul. 3, 2007; 11/832,163, filed Aug. 1, 2007; 11/832,197, filed on Aug. 1, 2007; the entire disclosure of each of these references is hereby incorporated herein by reference.

In a particular embodiment, the present invention provides a golf ball comprising:

- 65 (a) a fluid-filled center,
- (b) a first outer core layer formed from a low modulus HNP composition,

- (c) a second outer core layer formed from a high modulus HNP composition, and
- (d) a cover having one or more layers.

In a particular aspect of this embodiment, the center has a diameter within a range having a lower limit of 0.250 or 0.500 or 0.600 or 0.750 or 0.800 or 1.000 or 1.100 inches and an upper limit of 1.300 or 1.400 or 1.510 or 1.530 or 1.550 or 1.570 or 1.580 inches. In another particular aspect of this embodiment, the first outer core layer has a thickness within a range having a lower limit of 0.020 or 0.025 or 0.032 or 0.050 or 0.075 or 0.100 or 0.125 inches and an upper limit of 0.150 or 0.175 or 0.200 or 0.220 or 0.250 or 0.280 or 0.300 inches. In another particular aspect of this embodiment, the second outer core layer has a thickness within a range having a lower limit of 0.020 or 0.025 or 0.032 inches and an upper limit of 0.310 or 0.440 or 0.560 inches; or the second outer core layer has a thickness such that the overall core diameter is within a range having a lower limit of 1.450 or 1.500 or 1.510 or 1.530 or 1.550 inches and an upper limit of 1.560 or 1.570 or 1.580 or 1.590 or 1.600 or 1.620 inches. In another particular aspect of this embodiment, the cover has an overall thickness within the range having a lower limit of 0.020 or 0.025 or 0.030 or 0.060 inches and an upper limit of 0.065 or 0.080 or 0.090 or 0.110 inches; or the cover includes an inner cover layer and outer cover layer, wherein the inner cover layer has a thickness within a range having a lower limit of 0.010 or 0.015 inches and an upper limit of 0.035 or 0.040 or 0.045 or 0.050 or 0.055 or 0.750 or 0.100 inches and the outer cover layer has a thickness within a range having a lower limit of 0.010 or 0.015 inches and an upper limit of 0.035 or 0.040 or 0.045 or 0.050 or 0.055 or 0.750 or 0.115 inches. In another particular aspect of this embodiment, the core has an overall core compression of 100 or less, or less than 100, or the core has an overall core compression within a range having a lower limit of 20 and an upper limit of 50 or 80 or 90 or 100. In yet another particular aspect of this embodiment, the low modulus HNP of the first outer core layer has a modulus within the range having a lower limit of 1,000 or 5,000 or 10,000 psi and an upper limit of 17,000 or 28,000 or 30,000 or 50,000 psi and the high modulus HNP of the second outer core layer has a modulus within the range having a lower limit of 45,000 or 55,000 or 60,000 psi and an upper limit of 72,000 or 75,000 or 100,000 or 150,000 psi.

In another particular embodiment, the present invention provides a golf ball comprising:

- (a) a fluid-filled center,
- (b) a first outer core layer formed from a high modulus HNP composition,
- (c) a second outer core layer formed from a low modulus HNP composition, and
- (d) a cover having one or more layers.

In a particular aspect of this embodiment, the center has a diameter within a range having a lower limit of 0.250 or 0.500 or 0.600 or 0.750 or 0.800 or 1.000 or 1.100 inches and an upper limit of 1.300 or 1.400 or 1.510 or 1.530 or 1.550 or 1.570 or 1.580 inches. In another particular aspect of this embodiment, the first outer core layer has a thickness within a range having a lower limit of 0.020 or 0.025 or 0.032 or 0.050 or 0.075 or 0.100 or 0.125 inches and an upper limit of 0.150 or 0.175 or 0.200 or 0.220 or 0.250 or 0.280 or 0.300 inches. In another particular aspect of this embodiment, the second outer core layer has a thickness within a range having a lower limit of 0.020 or 0.025 or 0.032 inches and an upper limit of 0.310 or 0.440 or 0.560 inches; or the second outer core layer has a thickness such that the overall core diameter is within a range having a lower limit of 1.450 or 1.500 or 1.510 or 1.530 or 1.550 inches and an upper limit of 1.560 or

1.570 or 1.580 or 1.590 or 1.600 or 1.620 inches. In another particular aspect of this embodiment, the cover has an overall thickness within the range having a lower limit of 0.020 or 0.025 or 0.030 or 0.060 inches and an upper limit of 0.065 or 0.080 or 0.090 or 0.110 inches; or the cover includes an inner cover layer and outer cover layer, wherein the inner cover layer has a thickness within a range having a lower limit of 0.010 or 0.015 inches and an upper limit of 0.035 or 0.040 or 0.045 or 0.050 or 0.055 or 0.750 or 0.100 inches and the outer cover layer has a thickness within a range having a lower limit of 0.010 or 0.015 inches and an upper limit of 0.035 or 0.040 or 0.045 or 0.050 or 0.055 or 0.750 or 0.115 inches. In another particular aspect of this embodiment, the core has an overall core compression of 100 or less, or less than 100, or the core has an overall core compression within a range having a lower limit of 20 and an upper limit of 50 or 80 or 90 or 100. In yet another particular aspect of this embodiment, the low modulus HNP of the second outer core layer has a modulus within the range having a lower limit of 1,000 or 5,000 or 10,000 psi and an upper limit of 17,000 or 28,000 or 30,000 or 50,000 psi and the high modulus HNP of the first outer core layer has a modulus within the range having a lower limit of 45,000 or 55,000 or 60,000 psi and an upper limit of 72,000 or 75,000 or 100,000 or 150,000 psi.

In addition to the materials disclosed above, any of the core or cover layers may comprise one or more of the following materials: thermoplastic elastomer, thermoset elastomer, synthetic rubber, thermoplastic vulcanizate, copolymeric ionomer, terpolymeric ionomer, polycarbonate, polyolefin, polyamide, copolymeric polyamide, polyesters, polyester-amides, polyether-amides, polyvinyl alcohols, acrylonitrile-butadiene-styrene copolymers, polyarylate, polyacrylate, polypheylene ether, impact-modified polyphenylene ether, high impact polystyrene, diallyl phthalate polymer, metallocene-catalyzed polymers, styrene-acrylonitrile (SAN), olefin-modified SAN, acrylonitrile-styrene-acrylonitrile, styrene-maleic anhydride (S/MA) polymer, styrenic copolymer, functionalized styrenic copolymer, functionalized styrenic terpolymer, styrenic terpolymer, cellulose polymer, liquid crystal polymer (LCP), ethylene-propylene-diene rubber (EPDM), ethylene-vinyl acetate copolymer (EVA), ethylene propylene rubber (EPR), ethylene vinyl acetate, polyurea, and polysiloxane. Suitable polyamides for use as an additional material in compositions disclosed herein also include resins obtained by: (1) polycondensation of (a) a dicarboxylic acid, such as oxalic acid, adipic acid, sebacic acid, terephthalic acid, isophthalic acid or 1,4-cyclohexanedicarboxylic acid, with (b) a diamine, such as ethylenediamine, tetramethyleneediamine, pentamethyleneediamine, hexamethylene diamine, or decamethylene diamine, 1,4-cyclohexyldiamine or m-xylylenediamine; (2) a ring-opening polymerization of cyclic lactam, such as  $\epsilon$ -caprolactam or  $\omega$ -laurolactam; (3) polycondensation of an aminocarboxylic acid, such as 6-aminocaproic acid, 9-aminononanoic acid, 11-aminoundecanoic acid or 12-aminododecanoic acid; or (4) copolymerization of a cyclic lactam with a dicarboxylic acid and a diamine. Specific examples of suitable polyamides include Nylon 6, Nylon 66, Nylon 610, Nylon 11, Nylon 12, copolymerized Nylon, Nylon MXD6, and Nylon 46.

Other preferred materials suitable for use as an additional material in golf ball compositions disclosed herein include Skypel polyester elastomers, commercially available from SK Chemicals of South Korea; Septon® diblock and triblock copolymers, commercially available from Kuraray Corporation of Kurashiki, Japan; and Kraton® diblock and triblock copolymers, commercially available from Kraton Polymers LLC of Houston, Tex.

Ionomers are also well suited for blending with compositions disclosed herein. Suitable ionomeric polymers include  $\alpha$ -olefin/unsaturated carboxylic acid copolymer- or terpolymer-type ionomeric resins. Copolymeric ionomers are obtained by neutralizing at least a portion of the carboxylic groups in a copolymer of an  $\alpha$ -olefin and an  $\alpha,\beta$ -unsaturated carboxylic acid having from 3 to 8 carbon atoms, with a metal ion. Terpolymeric ionomers are obtained by neutralizing at least a portion of the carboxylic groups in a terpolymer of an  $\alpha$ -olefin, an  $\alpha,\beta$ -unsaturated carboxylic acid having from 3 to 8 carbon atoms, and an  $\alpha,\beta$ -unsaturated carboxylate having from 2 to 22 carbon atoms, with a metal ion. Examples of suitable  $\alpha$ -olefins for copolymeric and terpolymeric ionomers include ethylene, propylene, 1-butene, and 1-hexene. Examples of suitable unsaturated carboxylic acids for copolymeric and terpolymeric ionomers include acrylic, methacrylic, ethacrylic,  $\alpha$ -chloroacrylic, crotonic, maleic, fumaric, and itaconic acid. Copolymeric and terpolymeric ionomers include ionomers having varied acid contents and degrees of acid neutralization, neutralized by monovalent or bivalent cations as disclosed herein. Examples of commercially available ionomers suitable for blending with compositions disclosed herein include Surlyn® ionomer resins, commercially available from E. I. du Pont de Nemours and Company, and Iotek® ionomers, commercially available from ExxonMobil Chemical Company.

Silicone materials are also well suited for blending with compositions disclosed herein. Suitable silicone materials include monomers, oligomers, prepolymers, and polymers, with or without adding reinforcing filler. One type of silicone material that is suitable can incorporate at least 1 alkenyl group having at least 2 carbon atoms in their molecules. Examples of these alkenyl groups include, but are not limited to, vinyl, allyl, butenyl, pentenyl, hexenyl, and decenyl. The alkenyl functionality can be located at any location of the silicone structure, including one or both terminals of the structure. The remaining (i.e., non-alkenyl) silicon-bonded organic groups in this component are independently selected from hydrocarbon or halogenated hydrocarbon groups that contain no aliphatic unsaturation. Non-limiting examples of these include: alkyl groups, such as methyl, ethyl, propyl, butyl, pentyl, and hexyl; cycloalkyl groups, such as cyclohexyl and cycloheptyl; aryl groups, such as phenyl, tolyl, and xylyl; aralkyl groups, such as benzyl and phenethyl; and halogenated alkyl groups, such as 3,3,3-trifluoropropyl and chloromethyl. Another type of suitable silicone material is one having hydrocarbon groups that lack aliphatic unsaturation. Specific examples include: trimethylsiloxy-endblocked dimethylsiloxane-methylhexenylsiloxane copolymers; dimethylhexenylsiloxy-endblocked dimethylsiloxane-methylhexenylsiloxane copolymers; trimethylsiloxy-endblocked dimethylsiloxane-methylvinylsiloxane copolymers; trimethylsiloxy-endblocked methylphenylsiloxane-dimethylsiloxane-methylvinylsiloxane copolymers; dimethylvinylsiloxyl-endblocked dimethylpolysiloxanes; dimethylvinylsiloxyl-endblocked dimethylsiloxane-methylvinylsiloxane copolymers; dimethylvinylsiloxyl-endblocked methylphenylsiloxanes; dimethylvinylsiloxyl-endblocked methylphenylsiloxane-dimethylsiloxane-methylvinylsiloxane copolymers; and the copolymers listed above wherein at least one group is dimethylhydroxysiloxyl. Examples of commercially available silicones suitable for blending with compositions disclosed herein include Silastic® silicone rubber, commercially available from Dow Corning Corporation of Midland, Mich.; Blensil® silicone rubber, commercially available from General Electric Company of Waterford, N.Y.;

and Elastosil® silicones, commercially available from Wacker Chemie AG of Germany.

Other types of copolymers can also be added to the golf ball compositions disclosed herein. For example, suitable copolymers comprising epoxy monomers include styrene-butadiene-styrene block copolymers in which the polybutadiene block contains an epoxy group, and styrene-isoprene-styrene block copolymers in which the polyisoprene block contains epoxy. Examples of commercially available epoxy functionalized copolymers include ESBS A1005, ESBS A1010, ESBS A1020, ESBS AT018, and ESBS AT019 epoxidized styrene-butadiene-styrene block copolymers, commercially available from Daicel Chemical Industries, Ltd. of Japan.

Ionomeric compositions used to form golf ball layers of the present invention can be blended with non-ionic thermoplastic resins, particularly to manipulate product properties. Examples of suitable non-ionic thermoplastic resins include, but are not limited to, polyurethane, poly-ether-ester, polyamide-ether, polyether-urea, Pebax® thermoplastic polyether block amides commercially available from Arkema Inc., styrene-butadiene-styrene block copolymers, styrene (ethylene-butylene)-styrene block copolymers, polyamides, polyesters, polyolefins (e.g., polyethylene, polypropylene, ethylene-propylene copolymers, ethylene-(meth)acrylate, ethylene-(meth)acrylic acid, functionalized polymers with maleic anhydride grafting, epoxidation, etc., elastomers (e.g., EPDM, metallocene-catalyzed polyethylene) and ground powders of the thermoset elastomers.

Also suitable for forming the outer core layers are the compositions having high COR when formed into solid spheres disclosed in U.S. Patent Application Publication No. 2003/0130434 and U.S. Pat. No. 6,653,382, the entire disclosures of which are hereby incorporated herein by reference.

### 35 Additional Examples of Suitable HNPs

The HNPs of the table below have been found to be particularly useful as the low modulus HNP and/or the high modulus HNP of the present invention.

40

| Example | cation source | Flexural Modulus*, psi | Hardness**, Shore C (18 day) | Hardness**, Shore D (annealed) |
|---------|---------------|------------------------|------------------------------|--------------------------------|
| 45 1    | Ca/Mg         | 71,600                 | 88                           | 57                             |
| 2       | Ca/Li         | 70,300                 | 89                           | 58                             |
| 3       | Ca            | 70,100                 | 92                           | 60                             |
| 4       | Ca/Zn         | 60,400                 | 88                           | 58                             |
| 5       | Mg            | 38,300                 | 84                           | 52                             |
| 6       | Mg            | 27,600                 | 84                           | 52                             |
| 50 7    | Mg            | 16,300                 | 78                           | 45                             |
| 8       | Mg            | 10,600                 | 70                           | 40                             |
| 9       | Mg            | 10,400                 | 69                           | 39                             |

\*Flexural modulus was measured according to ASTM D790-03 Procedure B.

\*\*Hardness was measured according to ASTM D2240.

55

In embodiments of the present invention directed to a golf ball having a first outer core layer formed from a low modulus HNP composition, Examples 6-9 are particularly suitable for use as the low modulus HNP composition.

60

In embodiments of the present invention directed to a golf ball having a second outer core layer formed from a low modulus HNP composition, Examples 5-9 are particularly suitable for use as the low modulus HNP composition.

65

In embodiments of the present invention directed to a golf ball having a first outer core layer formed from a high modulus HNP composition, Examples 1-6 are particularly suitable for use as the high modulus HNP composition.

## 19

In embodiments of the present invention directed to a golf ball having a second outer core layer formed from a high modulus HNP composition, Examples 1-4 are particularly suitable for use as the high modulus HNP composition.

When numerical lower limits and numerical upper limits are set forth herein, it is contemplated that any combination of these values may be used.

All patents, publications, test procedures, and other references cited herein, including priority documents, are fully incorporated by reference to the extent such disclosure is not inconsistent with this invention and for all jurisdictions in which such incorporation is permitted.

While the illustrative embodiments of the invention have been described with particularity, it will be understood that various other modifications will be apparent to and can be readily made by those of ordinary skill in the art without departing from the spirit and scope of the invention. Accordingly, it is not intended that the scope of the claims appended hereto be limited to the examples and descriptions set forth herein, but rather that the claims be construed as encompassing all of the features of patentable novelty which reside in the present invention, including all features which would be treated as equivalents thereof by those of ordinary skill in the art to which the invention pertains.

What is claimed is:

1. A golf ball comprising a core and a cover, wherein the core comprises:

(a) a fluid mass at the center;  
 (b) a first outer core layer surrounding the fluid mass, wherein the first outer core layer is solid, non-wound, and formed from a low modulus HNP composition, the low modulus HNP composition comprising:  
 a highly neutralized ethylene/(meth)acrylic acid/alkyl (meth)acrylate copolymer having a modulus of from 1,000 psi to 50,000 psi; and

(c) a second outer core layer surrounding the first outer core layer, wherein the second outer core layer is solid, non-wound, and formed from a high modulus HNP composition, the high modulus HNP composition comprising:  
 a highly neutralized ethylene/(meth)acrylic acid copolymer having a modulus of from 25,000 psi to 150,000 psi;

wherein the modulus of the highly neutralized copolymer of the low modulus HNP composition is at least 10% less than the modulus of the highly neutralized copolymer of the high modulus HNP composition.

2. The golf ball of claim 1, wherein the highly neutralized ethylene/(meth)acrylic acid/alkyl (meth)acrylate copolymer of the first outer core layer is neutralized at least 80% by a cation source selected from the group consisting of metal ions and compounds of potassium, cesium, calcium, barium, manganese, copper, zinc, tin, and rare earth elements.

3. The golf ball of claim 1, wherein the first and second outer core layers have a combined thickness of from 0.04 inches to 0.56 inches.

4. The golf ball of claim 1, wherein the fluid mass has a specific gravity of from 1.3 to 1.55.

5. The golf ball of claim 1, wherein the fluid mass has a viscosity of from 100 to 1500 cps.

## 20

6. The golf ball of claim 1, wherein the golf ball additionally comprises a thin shell layer disposed between the center and the first outer core layer.

7. The golf ball of claim 1, wherein the core has a compression of 87 or less.

8. The golf ball of claim 1, wherein the first outer core layer has a moisture vapor transmission rate of 8 g-mil 100 in<sup>2</sup>/day or less.

9. The golf ball of claim 1, wherein the first outer core layer has a moisture vapor transmission rate of 2 g-mil 100 in<sup>2</sup>/day or less.

10. A golf ball comprising a core and a cover, wherein the core comprises:

(a) a fluid mass at the center;  
 (b) a first outer core layer surrounding the fluid mass, wherein the first outer core layer is solid, non-wound, and formed from a high modulus HNP composition, the high modulus HNP composition comprising:  
 a highly neutralized ethylene/(meth)acrylic acid copolymer having a modulus of from 25,000 psi to 150,000 psi; and

(c) a second outer core layer surrounding the first outer core layer, wherein the second outer core layer is solid, non-wound, and from a low modulus HNP composition, the low modulus HNP composition comprising:

a highly neutralized ethylene/(meth)acrylic acid/alkyl (meth)acrylate copolymer having a modulus of from 1,000 psi to 50,000 psi;

wherein the modulus of the highly neutralized copolymer of the low modulus HNP composition is at least 10% less than the modulus of the highly neutralized copolymer of the high modulus HNP composition.

11. The golf ball of claim 10, wherein the highly neutralized ethylene/(meth)acrylic acid/alkyl (meth)acrylate copolymer of the first outer core layer is neutralized at least 80% by a cation source selected from the group consisting of metal ions and compounds of potassium, cesium, calcium, barium, manganese, copper, zinc, tin, and rare earth elements.

12. The golf ball of claim 10, wherein the first and second outer core layers have a combined thickness of from 0.04 inches to 0.56 inches.

13. The golf ball of claim 10, wherein the fluid mass has a specific gravity of from 1.3 to 1.55.

14. The golf ball of claim 10, wherein the fluid mass has a viscosity of from 100 to 1500 cps.

15. The golf ball of claim 10, wherein the golf ball additionally comprises a thin shell layer disposed between the center and the first outer core layer.

16. The golf ball of claim 10, wherein the core has a compression of 87 or less.

17. The golf ball of claim 10, wherein the first outer core layer has a moisture vapor transmission rate of 8 g-mil 100 in<sup>2</sup>/day or less.

18. The golf ball of claim 10, wherein the first outer core layer has a moisture vapor transmission rate of 2 g-mil 100 in<sup>2</sup>/day or less.